# EUROPEAN PATENT APPLICATION

(11) **EP 1 837 885 A1**
(43) Date of publication of application: **26.09.2007**
(21) Application number: 07251195.9
(22) Date of filing: 21.03.2007
(51) Int. Cl.: H01B 3/10, H01B 7/29, H01B 7/295, H01B 3/44, H01B 7/02

(54) **Improvements in or relating to electric wiring**

(30) Priority: 24.03.2006 GB 0605918
(71) Applicant: Tyco Electronics UK Ltd., Dorcan Swindon SN3 5HH (GB)
(72) Inventor: Rodway, Giles, Calne, Wiltshire SN11 8DJ (GB)
(74) Representative: Khan, Mohammed Saiful Azam

(57) **Abstract**

The present invention provides an electric wire (100) comprising an electric conductor (110) surrounded by an inner (120) and an outer (130) insulating sheath layer, wherein the inner sheath layer (120) is formed into a sheath by extrusion to surround the electric conductor (110), and wherein the inner sheath layer (120) comprises an extruded matrix of particulate material (121) and binding material (122).

## Description

### Field of the Present Invention

The present invention relates to the field of electric wires used to conduct electrical signalling, for example, between electrical components. The present invention also relates to wires used to supply power, for example, wires used to connect a power supply to an electrical component. Such wires generally comprise an electrical conductor core encapsulated by one or more protective nonconductive layers. The term electric wire is used to encompass the term electric cable, the term cable often being used to refer to comparatively large wires.

The conductive core can be made from a variety of conductive materials, and may be formed from a single piece of conductive wire or a bunch of electrically conductive wires grouped/wound together. For example, in the case of electrical signalling wiring, the wires may comprise a core comprising a twisted pair of insulated electrical conductive material (e.g. copper), encapsulated inside a protective jacket.

Although specific embodiments of the present invention relate to high temperature electrical wiring, such as those used in the automotive industry for routings near manifolds, catalytic converters and diesel traps (i.e. high temperature continuous use applications), all aspects and embodiments of the present invention are not limited to such applications or operating conditions. Certain aspects and embodiments of the present invention can be applied to other industries and applications, and are not necessarily limited to use in such high temperature conditions.

### Background to the Present Invention

Let us consider an application in the automotive industry in which there is a significant demand for high temperature electrical wiring. Typically, in the case of routings close to exhaust manifolds, for example, electrical wiring may be required to be rated to operate at temperature in excess of 150°C (for 3000h, as in, for example the ISO 6722 automotive wire specification). In such applications; fluoropolymer wire insulation materials are frequently used, as these are among the few polymers capable of simultaneously meeting the mechanical, thermal, electrical and chemical resistance requirements.

The disadvantage of these fluoropolymer materials, such as ETFE, FEP, and PTFE (and other high temperature polymers), is that they are usually extremely expensive, often an order of magnitude more expensive per unit volume than the insulating materials of choice, such as PE, PP, and PVC, for lower temperature applications. Furthermore, these high temperature materials, although often over-specified for the applications for which they are used, are typically not suitable for blending with a high proportion of a lower cost "filler" material, to reduce the overall insulation cost per unit volume, as their filler acceptance is relatively poor.

For some applications, a reduction in the overall thickness of the insulation may be possible, thus saving insulation and hence cost. There are limitations on this technique, however, as insulation which is too thin becomes difficult to strip off the wire for termination, and for other applications, certain overall dimensions are required, e.g. to ensure that insulated wire of a particular gauge fits into standard grommets or seals.

Given the above constraints, one method which has been used in the past to reduce the proportion of fluoropolymer in wire insulation, whilst still maintaining some of its beneficial properties, has been to extrude the fluoropolymer insulation over a pre-extruded layer of a low cost polymeric insulation. In this way, this lower cost insulation, which would not itself meet the full requirements of the specification at a particular temperature, is protected by an outer layer of fluoropolymer. The most successful example of such a wire has been Tyco Electronics' "ACW" wire, widely used by the European automotive industry in 150°C rated applications since the late 1990s. This wire consists of a crosslinked polyethylene inner layer of insulation, covered by a fluoropolymer (in this particular case, polyvinylidene fluoride, or PVDF) outer layer (also known as a primary jacket, or "PJ").

Attempts to push such technologies to higher temperatures, principally 175°C or 200°C have, to date, been unsuccessful, due to the following failure mode under such conditions:
The polymeric inner wire layer, upon ageing at the higher temperature, becomes embrittled. At, or before, the time corresponding to the required service life, the inner layer embrittles to such an extent that it cracks into relatively large blocks of a stiff, embrittled material on flexing or bending. This, in turn, produces large stress concentrations in the outer layer (PJ), which causes it to tear, and thus exposes the copper conductor to the outside environment.

DE19729395, DE19728195, and EP0076560 all disclose fire resistant electric wires/cables comprising an electric conductor surrounded by inner and outer insulating sheath layers. Such fire resistant cables are designed to maintain circuit integrity after a fire, and make use of powder compositions contained between the inner and outer sheath layers to improve resistance to such high temperatures. However, the teachings of these documents do not relate to the use of powder compositions to form extruded sheaths.

### Summary of the Present Invention

According to a first aspect, the present invention provides an electric wire comprising an electric conductor surrounded by an inner and an outer insulating sheath layer, wherein the inner sheath layer is formed into a sheath by extrusion to surround the electric conductor, and wherein the inner sheath layer comprises an extruded matrix of particulate material and binding material.

The relative percentage composition (whether by volume or weight) of the inner layer allows sufficient structural integrity to allow the inner sheath to be extruded but yet allows the inner layer to crumble upon, for example, bending of the wire following extrusion.

The composition by volume and/or weight of the inner layer may be predominantly a particulate material, possibly up to 99% particulate material.

The composition of the inner layer may be at least 65% by weight/volume particulate material. The composition of the inner layer may be at least 70% by weight/volume particulate material. The composition of the inner layer may be at least 75% by weight/volume particulate material. The composition of the inner layer may be at least 80% by weight/volume particulate material.

The composition of the inner layer may be between 80%-85% by weight/volume particulate material. The composition of the inner layer may be between 85%-90% by weight/volume particulate material. The composition of the inner layer may be between 90%-95% by weight/volume particulate material. The composition of the inner layer may be between 95%-99% by weight/volume particulate material. The composition of the inner layer may be between 65%-95% by weight/volume particulate material. The composition of the inner layer may be between 65%-99% by weight/volume particulate material. The composition of the inner layer may be between 80%-90% by weight/volume particulate material.

The compositions quoted may be prior to extrusion and/or post extrusion.

The composition of the binding material of the inner layer may be a polymer or polymer blend.

The composition of the binding material of the inner layer may be a polymer or polymer blend selected from the list of EVA, PE, PVC, or PP.

The particulate material may be a refractory material.

The particulate material may be selected from the list magnesium hydroxide, talc, calcium carbonate, zinc sulphide, titanium dioxide, aluminium trihydrate, silica, alumina, antimony trioxide, or other inorganic (or organic) materials, or a blends of one or more of such materials.

The outer layer may be formed from a polymer.

The outer layer may be formed from a fluoropolymer selected from the list ETFE, FEP, PFA, MFA, ECTFE or PVDF or a fluoroelastomer.

The wire may be a high temperature automotive electric wire.

The outer layer may be a temperature resistant layer and the inner layer may be a friable layer.

The inner and outer layers may be immediately adjacent to one another.

The inner layer may be made from a material which is capable of remaining intact in a static application to provide electrical integrity of the wire even after the electric wire has been exposed to the high temperature.

The inner layer may be made from a material which is capable of remaining intact in a static application to provide electrical integrity of the wire even after the electric wire has been exposed to fire.

The inner layer may be made from a material which sinters when exposed to a high temperature to provide sufficient mechanical strength to maintain the electrical integrity of the wire even after the electric wire has been exposed to the high temperature.

The inner layer may be made from a material which sinters when exposed to a high temperature to provide sufficient mechanical strength to maintain the electrical integrity of the wire even after the electric wire has been exposed to the fire.

The inner layer and/or outer layer may be made from a material which forms a char upon exposure to a high temperature to maintain the mechanical strength of the inner and/or outer core at a sufficient level to maintain the electrical integrity of the wire.

The particulate material may comprise magnesium hydroxide.

The particulate material of the inner layer may be dimensioned and shaped to provide stress concentrations on the outer layer which do not tear the outer layer under one or more of operating/installation/maintenance conditions.

The wire may be arranged to not maintain circuit integrity under exposure to fire.

According to a second aspect, the present invention provides a method of manufacturing a wire according to the first aspect of the invention.

The present invention encompasses one or more aspects and or embodiments of the present invention in all possible combinations, whether or not specifically mentioned in that combination.

In one or more aspects and/or embodiments of the present invention, the failure mode described in the Background section above is avoided by using a friable core layer, which breaks up on bending after ageing, but into a smaller scale particulate or powdery form. Surprisingly, this inner layer, which is significantly weaker than a polymeric core layer at all times in the ageing cycle, does not lead to cracking of the outer (Polymer Jacket) layer. This is because the way in which the new inner layer breaks up avoids the high stress concentrations associated with large cracks.

The outer PJ layer is thus able to contain the powder, and to elongate in a uniform way to cover it on bending. By the present technique, rated temperatures for the composite (two layer) insulation equivalent to the rated temperature of the fluoropolymer when aged as a single wall insulation are achievable; e.g. 200°C in the case of crosslinked ETFE insulation. Suitable inner layer insulation materials comprise predominantly of inorganic filler materials (such as Mg(OH)₂), with relatively small amounts of polymer which act principally as a binder, but are sufficient to allow extrusion of the inner layer onto the conductive core. Additional process aids may be added to assist with the compounding and extrusion processes.

### Brief Description of the Figures

Specific embodiments of the present invention will now be described with reference to the following Figures in which :
Figure 1 illustrates a cross section though a wire according to a first embodiment of the present invention;
Figure 2 illustrates a cross section though a wire according to a second embodiment of the present invention;
Figure 3 illustrates a cross section though a wire according to a third embodiment of the present invention; and
Figure 4 illustrates a cross section though a wire according to a fourth embodiment of the present invention.

### Description of Specific Embodiments

Figures 1-4 illustrate four different embodiments of the present invention. Similar reference numerals have been used for similar constituents in each of the figures (e.g. 110, 210, 310, 410 are used to reference the conductive core in the four embodiments of the wire 100, 200, 300, 400 shown in the figures).

In a first embodiment (Figure 1), the wire 100 comprises a conductive core 110, which is surrounded by an inner sheath 120 formed from extruded particulate material 121 and binding material 122. The inner sheath 120 is protected by an immediately adjacent outer polymer protective sheath 130.

In a second embodiment (Figure 2), the wire 200 comprises two conductive cores 210 around each of which have been separately extruded inner particulate/binding agent sheaths 220. The two sheaths 220 are protected and held together by a single outer sheath 230.

In the above two embodiments, the inner sheath 120, 220 is shown to be immediately adjacent the conductive core 110, 210. However, in a third embodiment (Figure 3), another sheath 340 is placed between the inner sheath 320 and the core 310. Sheaths 340 and 330 may also be conveniently applied by extrusion.

In a fourth embodiment (Figure 4), the two adjacent particulate/binding agent sheaths 220 of the embodiment of Figure 2, may be a single particulate/binding agent sheath 420. Thus, a single inner sheath 420 isolates the two adjacent conductive cores 410 from one another.

In one specific embodiment, the present invention comprises an electrical conductive core surrounded by :
- an inner insulation layer comprising >65% by weight of magnesium hydroxide Mg(OH)₂ particulate material, the balance of the formulation consisting of polypropylene (PP) "binding" polymer, with process aids (e.g. zinc stearate) added in quantities necessary to assist compounding (i.e. the production of a compound by mixing ingredients);
- and an immediately adjacent outer insulating layer of ethylene tetrafluoroethylene (ETFE), containing similar stabilisers, colours, crosslinking promoters and other additives as are present in standard, commercially available single wall wires available for high temperature automotive applications.

Although the inner and outer layers in this embodiment are immediately adjacent to one another, in other embodiments, one or more layers may be placed between them. Although the above embodiment refers to the use of two insulation layers, the conductive core can be surrounded by more than two layers. The inner layer may or may not be immediately adjacent the conductive core.

Furthermore, in other embodiments, the inner layer may comprise >75%, and between 80-85% of the particulate material, such as Mg(OH)₂. The relative composition of particulate/binding material may be by volume rather than by weight, particularly for other particulate/binding material compositions.

The inner layer may be formed from other particulate materials, e.g. talc, calcium carbonate, zinc sulphide, titanium dioxide, aluminium trihydrate, silica, alumina, antimony trioxide, or other inorganic (or organic) filler materials, or blends of one or more of such materials.

The "binder" polymer and additives may be different from those listed above. For example, the binder polymer may be EVA, PE, PVC or other relatively low cost polymer co- or ter- polymers or polymer blend.

The materials for the inner (and outer) layer may be chosen to contribute to some characteristics for the wire, e.g. hot compression resistance, and/or flame retardance.

Other embodiments are possible, whereby the outer layer is another fluoropolymer, such as FEP, PFA, MFA, ECTFE or PVDF or a fluoroelastomer. The outer layer may be another high temperature material which is not a fluoropolymer material, for example, PEEK or Ultem. The outer layer may be formed from lower temperature polymer formulations. These may include polyester, TPEs, PP, crosslinked polyethylene, and would be particularly usefeul where other properties (e.g. circuit integrity after burning the cable, or reduced stiffness or cost compared to single layer constructions) are required.

In general terms, the inner insulation layer is formulated such that it is "friable", i.e. it easily breaks up into small particles or a powder when subject to a mechanical stress (e.g. flexing or impact), but holds together during manufacturing operations or in static applications. This combination of properties can be achieved, for example, by putting a certain range of extremely high inorganic filler/particulate material (typically >70% by volume/weight) into a matrix of polymeric material.

The outer insulation layer, is made from a more conventional polymer formulation (with the usual additives such as stabilizers, crosslinking promoters etc as necessary), to provide the overall insulation with its mechanical integrity, chemical resistance, and electrical insulation, in normal operating conditions.

The above construction has potential advantages over existing products, in several applications. For example, in high temperature automotive wires, the construction allows dimensional and functional requirements to be met at much lower cost than is possible with traditional constructions. This is because the high-cost fluoropolymer insulations are partially replaced by a much lower cost inner layer. The problems (principally crack propagation from the inner layer to the outer, after thermal ageing, causing failure of both layers) associated with conventional dual wall constructions, which are made from just a low cost polymeric inner layer, are avoided by the powdery/particulate nature of the inner layer in the present invention. Similarly other specialized wire types, where one layer is of a very expensive (or very stiff) material, may benefit from this approach.

In the case of automotive high temperature applications (for example, high continuous service temperatures of 3000h at 200°C), embodiments of the present invention fulfil the dimensional and specification requirements of high temperature automotive wires at minimum cost, by using the minimum amount of (expensive) fluoropolymer insulation, and retaining the ability to extrude both layers.

This is achieved by using a comparatively cheap inner layer, having a high concentration of particulate material compared to binding agent, designed to have no structural function other than to be an extrudable filler, and to be "benign", when it cracks, to the (structural) outer layer. This is because, if a conventional low cost polymer material were used as the inner layer, the material would typically break into large, glassy chunks after ageing, rupturing the outer layer on bending. However, if just a powder were used as the inner material, the product would not be extrudable, and hence could not be manufactured economically. Such arrangements therefore can provide cheaper automotive wire, which still meets the high temperature specification requirements.

The term high temperature can be for operating conditions above 50°C, above 100°C, above 150°C, above 200°C, above 250°C, above 300°C, above 350°C and/or for operating conditions between 50°C-100°C, between 100°C-150°C, between 150°C-200°C, between 200°C-250°C, between 250°C-300°C, between 300°C-350°C, between 100°C-200°C, between 200°C-300°C, and/or between 300°C-400°C. The term high temperature may be used for comparatively lower operating temperatures in the case of longer service life requirements.

The composition of the inner layer is deliberately designed to be friable (i.e. to crumble easily, for example, under pressure from fingers, or on bending, but still be extrudable). Thus, it would typically be full of cracks at all times in service, and in certain compositions, may possibly fall off the wire after a fire. Most insulation would melt, char, vaporise or fall off the wire during/after a fire. In fact, depending on the materials, the inner layer might form a stable char layer, possibly together with the outer layer, or the filler particles might sinter together.

The outer layer, an extruded polymer, must provide electrical, mechanical etc properties in service, but may not necessarily be expected to remain intact (nor hold the core together) after a fire.

In the present invention, the failure mode described in the background section of the present specification, is avoided by using a friable inner layer, which breaks up on bending after ageing, but into a smaller scale particulate or powdery form. Surprisingly, this inner layer, which is significantly weaker than a polymeric core layer at all times in the ageing cycle, does not lead to cracking of the outer (PJ) layer. This is because the way in which the new inner layer material breaks up avoids the high stress concentrations associated with large cracks. The PJ layer is thus able to contain the powder, and to elongate in a uniform way to cover it on bending. By the present technique, rated temperatures for the composite (two layer) insulation equivalent to the rated temperature of the fluoropolymer when aged as a single wall insulation are achievable; e.g. 200°C in the case of crosslinked ETFE insulation.

Suitable inner layer insulation materials identified to date consist predominantly of inorganic filler materials (such as Mg(OH)₂), with relatively small amounts of polymer which act principally as a binder, but are sufficient to allow extrusion of the inner layer onto the conductive core. Additionally, process aids may be added to assist with the compounding and extrusion processes.

To form the wire, both the inner and outer layers are extruded onto the central conductor. This can be done by appropriately adapted standard extrusion processes used for making wires. The wires according to the present invention can also be made by appropriately adapted pressure, tube, tandem or co-extrusion processes. The particulate and binding material may be compounded, and then the resulting compound pelletised in a separate step prior to wire extrusion. During wire extrusion, the compound pellets can then be fed into an extruder. In the wire extrusion step, the pelletised compound is re-melted and extruded around the conductor to form a sheath.

It is apparent that the particulates have a degree of high temperature resistance to remain as particulate material. Specifically, the particulate material has a melting point which is higher than the pelletisation/extrusion temperature used to formed the inner layer. The binding material has a melting point which is lower than the pelletisation/extrusion temperature used to formed the inner layer.

The sheaths in the wires according to the present invention can be of various thicknesses. For example, it has been possible to obtain an inner sheath 120 with a thickness of 0.25-0.35mm, and the outer sheath 130 with a thickness of 1.1-0.13mm using a 85%wt magnesium hydroxide with mesh size 325. The particulate material 121, 221, 321, 421 can have various sizes, shapes and distributions throughout the extruded inner sheath 120, 220, 320, 420.

Certain embodiments may also be useful in fire-resistant cable/wire applications. Currently, in some such applications, refractory tape, which is wrapped around the conductive core, forms the inner insulation layer and provides circuit integrity under fire conditions. In certain embodiments of the present invention, a refractory particulate material is held together by a binding agent and is used to form the inner layer. Such an arrangement may still provide the circuit integrity which is required in fire-resistant applications. Furthermore, any microcracks, which are formed in such an inner layer, may be reduced by a sintering process, which would occur under exposure to fire. Thus, even if the outer layer were burnt away, some circuit resistance may still be provided by such a sintered inner layer. The outer layer may form a char upon burning. There are embodiments of the present invention which do not provide circuit integrity under fire.

One or more embodiments of the present invention in all various combinations are within the scope of the present invention, whether or not they are specifically mentioned or claimed in that combination.

## Claims

1. An electric wire comprising an electric conductor surrounded by an inner and an outer insulating sheath layer, wherein the inner sheath layer is formed into a sheath by extrusion to surround the electric conductor, and wherein the inner sheath layer comprises an extruded matrix of particulate material and binding material.

2. An electric wire as claimed in claim 1, wherein the composition of the inner layer is at least 70% by weight/volume particulate material.

3. An electric wire as claimed in claim 1, wherein the composition of the inner layer is between 80%-95% by weight/volume particulate material.

4. An electric wire as claimed in claim 1, wherein the composition of the binding material of the inner layer is a polymer or polymer blend.

5. An electric wire as claimed in claim 1, wherein the outer layer is a temperature resistant layer and the inner layer is a friable layer.

6. An electric wire as claimed in claim 1, wherein the inner and outer layers are immediately adjacent to one another.

7. An electric wire as claimed in claim 1, wherein the inner layer is made from a material which is capable of remaining intact in a static application to provide electrical integrity of the wire even after the electric wire has been exposed to the high temperature.

8. An electric wire as claimed in claim 1, wherein the inner layer is made from a material which is capable of remaining intact in a static application to provide electrical integrity of the wire even after the electric wire has been exposed to fire.

9. An electric wire as claimed in claim 1, wherein the inner layer is made from a material which sinters when exposed to a high temperature to provide sufficient mechanical strength to maintain the electrical integrity of the wire even after the electric wire has been exposed to the high temperature.

10. An electric wire as claimed in claim 1, wherein the inner layer is made from a material which sinters when exposed to a high temperature to provide sufficient mechanical strength to maintain the electrical integrity of the wire even after the electric wire has been exposed to the fire.

11. An electric wire as claimed in claim 1, wherein the inner layer and/or outer layer is made from a material which forms a char upon exposure to a high temperature to maintain the mechanical strength of the inner and/or outer core at a sufficient level to maintain the electrical integrity of the wire.

12. An electric wire as claimed in claim 1, wherein the particulate material comprises magnesium hydroxide.

13. An electric wire as claimed in claim 1, wherein the particulate material of the inner layer are dimensioned and shaped to provide stress concentrations on the outer layer which do not tear the outer layer under one or more of operating/installation/maintenance conditions.

14. An electric wire as claimed in claim 1, wherein the wire is arranged to not maintain circuit integrity under exposure to fire.

15. An electric wire as hereinbefore described with reference to the accompanying figures.
